

[54] DIFFUSION BONDED CATHODE FOR  
ELECTRON DISCHARGE DEVICE

[75] Inventors: **John J. Decker; Donald R. Kerstetter**, both of Emporium, Pa.

[73] Assignee: **GTE Sylvania Incorporated**, Stamford, Conn.

[22] Filed: **May 18, 1973**

[21] Appl. No.: **361,830**

[52] U.S. Cl. .... **29/25.14**; 29/494; 313/270

[51] Int. Cl.<sup>2</sup> .... **H01J 9/00**; B23K 31/02

[58] Field of Search .... 29/25.13, 25.14, 191, 484, 29/498, 501, 502, 488, 494; 313/270

[56] References Cited

UNITED STATES PATENTS

|           |         |                     |            |
|-----------|---------|---------------------|------------|
| 2,708,249 | 5/1955  | Pryslak .....       | 29/25.16 X |
| 3,085,175 | 3/1963  | Knauf, Jr. ....     | 313/270    |
| 3,214,626 | 10/1965 | Larson .....        | 313/270    |
| 3,333,141 | 7/1967  | Lemmens et al. .... | 313/346 R  |
| 3,667,110 | 6/1972  | Gwyn, Jr. ....      | 29/488 X   |

OTHER PUBLICATIONS

B. R. Garrett et al., "Broad Applications of Diffusion Bonding," NASA CR-409, March 1966, pp. 19-26.

Primary Examiner—Roy Lake

Assistant Examiner—James W. Davie

Attorney, Agent, or Firm—Norman J. O'Malley; William H. McNeill; Donald R. Castle

[57]

ABSTRACT

A method of fabricating cathodes for electron discharge devices wherein the cathodes comprise a hollow tubular stack and a substantially cup-shaped top cap fitted over one end of the stack. The method comprises thoroughly cleaning the stack and cap such as by degreasing and water washing and then fitting the cap to the stack and firing first in air at a temperature of about 500-600°C and then in hydrogen at a temperature of at least 1,100°C whereby a diffusion bond is formed between the cap and the stack.

2 Claims, 2 Drawing Figures





Fig. 1



Fig. 2

## DIFFUSION BONDED CATHODE FOR ELECTRON DISCHARGE DEVICE

### BACKGROUND OF THE INVENTION

This invention relates to cathodes for electron discharge devices and more particularly to cathodes for cathode ray tubes. Such cathodes generally comprise a hollow tubular stack or body portion having a cup-shaped top cap bonded or otherwise affixed to one end thereof. In the past it has been the practice to weld the top cap to the stack in one or more places. While this procedure has worked well for many years it is costly and time consuming and introduces other problems as well. One of the major ones of these problems is the fact that the weld between a wall of the top cap and the stack is seldom smooth, and often introduces burrs or protrusions which can subsequently break off during tube operation. Furthermore, with the current trend toward high voltage operation in cathode ray tubes any protrusions or unevenness formed on the cathode makes it very subject to disruptive arcs.

Therefore, it would be very advantageous if a method of bonding a top cap to the stack could be found which obviated the above-cited disadvantages.

### OBJECTS AND SUMMARY OF THE INVENTION

It is, therefore, an object of this invention to obviate the above-cited disadvantages of the prior art method.

It is another object of the invention to enhance the fabrication of electron discharge device cathodes.

Yet another object of the invention is the provision of a method of attaching top caps to stacks which method does not utilize welding and which introduces no uneven spots or protrusions or weld contamination into the cathode assembly.

These objects are achieved in one aspect of the invention by the provision of a method which utilizes diffusion bonding of the top cap to the stack. To achieve this method it is necessary that the parts; i.e., the top cap and the stack be extremely clean. This can be achieved by first degreasing the cathode top cap and stack and can also include washing in water to remove any contaminating salts. Also, a high degree of precision in the fitting of the parts is required. This degree of precision is accomplished by having the internal diameter of the top cap the same as or just slightly larger than the outside diameter of the stack.

After cleaning, the top cap is fitted over one end of the stack, preferably under pressure of about 15 pounds. The now assembled cap and stack are then first fired in air to oxidize any volatile contaminants thereon and then second fired in a reducing atmosphere, generally hydrogen, at a temperature sufficiently high to form a diffusion bond between the top cap and the stack. While the oxidizing firing can take place at a temperature of about 500°-600°C the final or second firing in the reducing atmosphere should be accomplished at a temperature of about 1,100°C for at least one minute. Under these conditions the top cap is firmly bonded to the stack as by a diffusion bond.

The phenomenon being exhibited by this method has long been known to exist. That is, high temperature firing of super clean parts has generally resulted in a number of the parts sticking together. However, this in the past has always been a troublesome aspect of the firing procedures and it is believed that this is the first known practical use of the phenomenon.

### BRIEF DESCRIPTION OF THE DRAWINGS

FIG. 1 is an elevational view of a cathode, with parts broken away which can be fabricated by this method.

FIG. 2 is a flow diagram of the basic process of this invention.

### DESCRIPTION OF THE PREFERRED EMBODIMENTS

For a better understanding of the present invention, together with other and further objects, advantages and capabilities thereof, reference is made to the following disclosure and appended claims in conjunction with the above-described drawings.

Referring now to the drawings with greater particularity, in FIG. 1 there is shown a cathode assembly 10 which is comprised of a hollow tubular stack 12 and a top cap 14 bonded thereto. The top cap 14 is generally cup-shaped and fits tightly over one end of stack 12. It will be observed from a study of the figure that no additional bonding material is utilized between the two pieces. Only a tight fit and a high firing temperature are necessary to achieve a thermal diffusion bond.

Both the stack and top cap are formulated or fabricated from more or less conventional cathode materials: that is, nickel or nickel alloys containing at least about 95% nickel. The process works well with all known cathode materials.

The method is accomplished by first forming the stack by any known tubular forming technique; and the top cap also is fabricated by any known techniques such as die drawing. After the stack and cap are formed they are cleaned, as by degreasing to remove any organic contaminating materials and can then be water

washed to remove any salts that may be thereon. Ultrasonic cleaning is also a desirable cleaning technique. After cleaning, the cap is fitted to the stack, and a tight fit is preferable. Such a tight fit, of course, is accomplished by fabricating the internal diameter of the top

cap so that it is the same as or only slightly larger than the outside diameter of the stack. After the cap and stack are fitted together they are first fired in air to oxidize any volatile contaminants that may have been picked up and this firing is accomplished at a temperature of about 500°-600°C. After the oxidizing firing the cathode assembly is fired in a reducing atmosphere such as hydrogen at a temperature sufficiently high to form a diffusion bond between the top cap and the stack. The temperature of this firing should be about 1,100°C for at least one minute and preferably about 3 minutes. After the final firing it is found that the top cap is diffusion bonded to the stack in an extremely clean manner wherein no protrusions or burrs have been introduced.

At this stage the cathode is ready to have emissive material applied thereto.

It will be seen from the above that use of this process provides a very novel method of fabricating cathodes which is simple and inexpensive and eliminates the necessity of welding the top cap to the stack. It is very readily automated and produces extremely clean cathodes that can be operated in tubes employing extremely high anode voltages; that is, in the neighborhood of 30,000 volts, without causing noticeable arcing.

While there has been shown and described what is at present considered the preferred embodiment of the

invention, it will be apparent to those skilled in the art that various changes and modifications can be made therein without departing from the scope of the invention as defined by the appended claims.

What is claimed is:

1. A method of fabricating cathodes for electron discharge devices, said cathodes comprising a hollow tubular stack and a substantially cup-shaped top cap fitted over one end of said stack and affixed thereto, said method comprising the steps of: forming said tubular stack from a nickel alloy containing at least about 95% nickel; forming said top cap from a nickel alloy containing at least about 95% nickel; said top cap having an internal diameter just large enough to fit over the ex-

ternal diameter of said stack; cleaning said stack and said top cap; drying said stack and top cap; fitting said top cap onto said stack to form a cathode assembly; firing said assembly in air to oxidize any volatile contaminants thereon at a temperature of above about 500°-600°C; and firing said assembly in a reducing atmosphere at a temperature sufficiently high to form a diffusion bond between said top cap and said stack, said cathode assembly reaching a temperature of about 10 1,100°C for at least one minute during said firing in said reducing atmosphere.

2. The method of claim 1 wherein said top cap is fitted to said stack with a pressure of about 15 pounds.

\* \* \* \* \*